

Nov. 7, 1939.

J. H. HOERN

2,178,724

VALVE TAPPET

Filed April 19, 1938



FIG. 1.



FIG. 3.

FIG. 2.



INVENTOR  
Joseph H. Hoern.  
BY  
Harness, Dickey & Pierce.  
ATTORNEYS.

## UNITED STATES PATENT OFFICE

2,178,724

## VALVE TAPPET

Joseph H. Hoern, Birmingham, Mich., assignor to  
Eaton Manufacturing Company, Cleveland,  
Ohio, a corporation of Ohio

Application April 19, 1938, Serial No. 202,928

7 Claims. (Cl. 123—90)

This invention relates to valve tappets for internal combustion engines and particularly to a valve tappet of the so-called barrel type, the principal object being the provision of a highly efficient tappet of this general type that is extremely economical to manufacture.

Objects of the invention include the provision of a barrel type valve tappet of hollow construction, the interior surfaces of which are permanently sealed against the escape of foreign matter therefrom; the provision of a valve tappet as above described formed from a plurality of independently formed parts; the provision of a hollow barrel type valve tappet the exterior surface of which is hardened throughout the major portion of its area, certain portions of the tappet being formed of hardenable steel and other portions of the tappet being formed of a material of essentially non-hardening characteristics but the outer surface of which has been carburized and subsequently heated and quenched to harden the same; the provision of a barrel type valve tappet including a relatively thin walled hollow central body portion together with opposite end portions welded thereto, the hollow central body portion comprising a piece of metal bent into cylindrical formation and welded together at the opposed edges thereof; and the provision of a hollow barrel type valve tappet having a hermetically sealed hollow interior and including an end member having a blind threaded opening therein threadably receiving an adjusting means.

The above being among the objects of the present invention, the same consists in certain novel features of construction and combinations of parts to be hereinafter described with reference to the accompanying drawing, and then claimed, having the above and other objects in view.

In the accompanying drawing which illustrates a suitable embodiment of the present invention and in which like numerals refer to like parts throughout the several different views,

Fig. 1 is a vertical sectional view taken axially through a valve tappet constructed in accordance with the present invention;

Fig. 2 is a horizontal sectional view taken transversely through the valve tappet shown in Fig. 1 as on the line 2—2 thereof;

Fig. 3 is an exploded view in side elevation of the various component parts going to make up the valve tappet shown in the previous views.

One disadvantage of barrel type valve tappets as heretofore constructed is that foreign material is inevitably found in the interior of the tappet and is liable to work out of it in service to the bearing surface between the tappet and its guiding bore and to various other bearing surfaces in internal combustion engines of which it forms a part, thus fostering the early destruction of such bearing surfaces. Such foreign material

may occur in the nature of chips, shavings or the like of the material from which the tappet is made resulting from a machining or other step in the manufacture of the tappet, it may occur as a result of cores or the like where the tappet is of cast construction, it may occur as scale where the tappet is of a type requiring a hardening operation during manufacture, it may occur as rust resulting from an intended cleaning operation on the tappet by aqueous solutions, or for a number of other different reasons. The present invention provides a tappet of this type which obviates the above disadvantage in that the hollow interior of the tappet is hermetically sealed at an early stage in its manufacture thus eliminating the possibility of any foreign material finding its way into the interior of the tappet and positively preventing the escape of any foreign material from the interior of the tappet in service.

In the quantity production of valve tappets by more or less specialized machinery, the ultimate cost of producing the tappets, as is true in connection with a great many other articles produced in quantity, depends to a large extent upon the cost of material going into the tappet rather than to the cost of the various steps of operation thereon. Accordingly, in valve tappets which are to be produced in large quantities it is desirable to construct them of the cheapest material possible consistent with the ability to obtain the desired characteristics in the finished product. With this end in view the present invention provides a construction by means of which certain portions of the tappet may be formed of the cheapest types of material, yet the finished product will have all of the desirable characteristics of equivalent types of valve tappets heretofore produced from more expensive materials and will have certain definite advantages in addition thereto. This is obtained in part by forming a part of the tappet from a relatively cheap grade of sheet metal and another part of the tappet from a relatively cheap grade of bar stock, these parts, in accordance with a more limited phase of the invention, being carburized during manufacture so that in a subsequent hardening step to which the entire tappet is subjected the surfaces will be hardened to a desired degree and yet the interior portions thereof will remain relatively soft so as to enable the tappet to withstand impact without breakage and will permit machining of certain parts thereof by the usual methods practiced on unhardened material after the tappets have passed through the hardening operation. In a broader aspect of the invention such parts, however, may be formed of a so-called "medium" carbon steel

that will be hardened to a greater or lesser extent upon heating and quenching.

Referring now to the drawing an illustrative embodiment of the tappet formed in accordance with the present invention is shown. This tappet comprises a cylindrical main body portion 10. While in the broader aspects of the invention the main body portion 10 may be formed from seamless steel tubing or even machined out from the solid in accordance with a more restricted phase of the invention, it is preferably formed from sheet metal bent into cylindrical shape and having its abutting edges welded as at 12 in Fig. 2. In constructing the main body portion 10 from welded sheet metal as described, strips of sheet metal of suitable width may be formed into elongated tubes with the opposite edges of the strip brought into abutting relation and welded together in accordance with certain conventional methods of forming steel tubes, pipes or the like, and then sections of the desired length cut off. On the other hand a rectangular piece of sheet metal of the dimensions required to make a hollow tube of the dimensions of the main body portion 10 may be simply rolled up to bring the opposite edges into abutting relationship and then welding said edges together. Intermediate its length the portion 10 is preferably provided with one or more peripheral grooves 11 adapted to retain a body of lubricant therein during operation.

One end of the main body portion 10 is provided with an end member indicated generally at 14 and comprising a cylindrical body portion 16 of a diameter materially less than the inner diameter of the main body portion 10 and a radially outwardly projecting central flange portion 18 intermediate the ends thereof. The flange portion 18 is of an outer diameter equal to the outer diameter of the main body portion 10 and is welded thereto as at 19, preferably by a suitable resistance welding operation. The main body portion 16 of the end member 14 is provided with a central threaded bore 20 extending axially inwardly thereof from the outer end and terminating short of the inner end of the main body portion 16 so as to constitute a blind threaded opening for reception of a clearance adjusting screw 22. That portion of the main body portion 16 outwardly of the flange 18 is flattened off on diametrically opposite sides to provide wrench receiving faces. The main body portion 16 is made of a minimum diameter consistent with proper support of the adjusting screw to be received in the opening 20, its inwardly projecting end thus being radially spaced from the inner walls of the main body portion 10. From this it will be understood that if the hole 20 were extended into open communication with the hollow interior of the tappet it would make it impossible to drain out any liquid employed in an attempt to wash out the interior of the tappet because of the pocket thus formed by such radial spacing, and the retention of such liquid would result in rusting of the interior walls of the tappet.

In the broader aspects of the present invention any suitable type of adjusting screw 22 may be employed, but the type shown is that disclosed and claimed in United States Letters Patent No. 2,035,055 granted March 24, 1936 to Harold I. Dyer and owned by the assignee of the present invention, it being of a self-locking type eliminating the necessity of employing a lock nut in connection therewith.

The opposite end of the main body portion 10 is closed by a disc-like end member 24 providing

a surface for contacting the usual valve lifting cam of an internal combustion engine as is well understood in the art. The end 24 is preferably of the same outer diameter as the main body portion 10 and is suitably welded thereto as at 25, preferably by a resistance type of weld.

It will be understood from the description thus far given that the tappet shown in the drawing is hollow, that the ends 14 and 24 in being welded to the main body portion 10 are hermetically sealed thereto at their points of connection, and that the main body portion 10 and end 24 are imperforate and that the only opening in the end 14 is a blind opening so that the hollow interior of the tappet is hermetically sealed. This prevents any possible escape of any foreign material such as that previously described from the interior of the tappet to the interior of a cooperating engine during service and thereby positively eliminates any ill effects which would otherwise occur from such escape.

The end member 24 which is adapted to bear against a valve operating cam is formed from a material which as a whole will be hardened to a desirable extent upon being heated and quenched. One steel which is suitable for this purpose and which is mentioned as illustrative of the general class of material from which the end member 24 may be formed is that known as SAE #52,100 having the following composition.

|            | Per cent      |
|------------|---------------|
| Carbon     | 0.95-1.10     |
| Manganese  | 0.20-0.50     |
| Phosphorus | maximum 0.030 |
| Sulphur    | do 0.035      |
| Chromium   | 1.20-1.50     |

Balance principally iron

This material when suitably hardened will have a Rockwell hardness of at least 55, C scale.

Another suitable type of steel for the end member 24 where the same is to be carburized is that known as SAE #3115 having the following composition.

|            | Per cent      |
|------------|---------------|
| Carbon     | 0.10-0.20     |
| Manganese  | 0.30-0.60     |
| Phosphorus | maximum 0.040 |
| Sulphur    | do 0.050      |
| Nickel     | 1.00-1.50     |
| Chromium   | 0.45-0.75     |

Balance principally iron

In the broader aspects of the invention, the main body portion 10 at least, and the end member 14 if desired, may be formed of a medium carbon steel that may be hardened by heating and quenching to a desired hardness, for instance, equal to 40 Rockwell, Scale C. As indicative of the types of steel which may be employed for the main body portion and end member 14 in such case, the composition of SAE steel No. 1035 is here set out as a matter of illustration of a satisfactory steel for this purpose.

|            | Per cent      |
|------------|---------------|
| Carbon     | 0.30-0.40     |
| Manganese  | 0.60-0.90     |
| Phosphorus | maximum 0.045 |
| Sulphur    | do 0.055      |

Balance principally iron

Where, as is preferable for the sake of cheapness, the main body portion 10 and end member 14 in accordance with a more limited phase of the present invention are formed from a type of steel that is not hardenable in and of itself by

70

75

heating and quenching, they may be formed of a type of steel such, for instance, as that known as SAE #1020 having the following composition.

|                          | Per cent      |
|--------------------------|---------------|
| 5 Carbon                 | 0.15-0.25     |
| Manganese                | 0.30-0.60     |
| Phosphorus               | maximum 0.045 |
| Sulphur                  | do 0.055      |
| Balance principally iron |               |

10 Where the parts 10 and 14 are formed of a material which is not hardenable in and of itself by simply heating and quenching, nevertheless the exterior surfaces thereof and particularly those surfaces thereof exposed to a sliding action 15 in the cooperating tappet bore of an engine in operation are hardened. This is accomplished by carburizing the exterior surfaces of these parts, as by packing in bone black and heating in accordance with conventional practice, to such an extent that after the ends 14 and 24 have 20 been welded to the main body portion 10 and the entire assembly is heated to a suitable temperature and quenched, not only will the end member 25 24 be hardened to the desired extent but in addition the surface of the main body portion 10 and end member 14, because of the added carbon absorbed by such surfaces during the carburization treatment, will also be hardened. As 30 will be understood by those skilled in the art the degree to which the surfaces of the members 10 and 14 may be hardened and the depth of the hardened skin or surface thereof will depend upon the particular type of carburizing treatment 35 to which these parts are subjected and the length of time to which they are subjected to such treatment, as well as the temperature to which the parts are heated prior to quenching. Preferably in such case the surfaces of the members 10 and 14 are carburized to such an extent 40 that when the entire assembly is heated to the temperature required to obtain the desired hardening of the end 24 upon subsequent quenching, the resulting hardness of the surface of the main body portion 10 will be in the neighborhood of 45 40 Rockwell, C scale, or higher. Moreover, where the end member 24 is formed of SAE #3150 steel or its equivalent, it likewise is carburized so that its working face will be hardened when heated and quenched, preferably to a hardness 50 of at least 60 Rockwell, or better. The particular manner of manufacturing the tappets herein shown to obtain the various features referred to forms no part of the present invention but constitutes the subject of my co-pending application 55 for Letters Patent of the United States for improvements in Method of making valve tappets, filed April 27, 1938 and serially numbered 204,692. In any event, regardless of the method of manufacture it will be observed that the tappet comprising the present invention has a hardened exterior surface and that the inner portions of the main body 10 and end member 14 is of relatively soft or at least unhardened nature which renders the tappet relatively resistant to rupture 60 under impact and desirable for that reason.

It will be understood that the particular embodiment of the invention illustrated and described is subject to various changes in details of construction without departing from the spirit 65 of the invention as defined in the appended claims.

What I claim is:

1. A valve tappet comprising a hollow cylindrical main body portion, an end member closing one end of said main body portion and welded

thereto, and a second end member received by the opposite end of said main body portion and welded thereto, the last mentioned end member being of relatively hard character and of uniform hardness therethrough, the surface areas of said main body portion and the first mentioned end member being of relatively hard character and said main body portion and said first mentioned end member being of relatively soft character except for said surfaces.

2. A hollow valve tappet comprising an imperforate hollow cylindrical main body portion, an imperforate end member secured and sealed to an end of said main body portion and having a blind threaded opening therein, a second imperforate end member secured and sealed to the opposite end of said main body portion, the last mentioned end member comprising material of relatively hard characteristics and of substantially uniform hardness therethrough, and said main body portion and the first mentioned end member having exposed outer surfaces of relatively hard character and inner portions of unhardened material.

3. A valve tappet comprising a sheet metal main body portion opposite edges of which are welded along the line extending longitudinally of said main body portion, end members secured to opposite ends of said main body portion, one of said end members being formed of relatively hard material of substantially uniform hardness throughout and the other of said end members and the main body portion having a relatively hard outer surface and a relatively soft interior body.

4. A valve tappet comprising a hollow cylindrical sheet metal body portion having a longitudinally extending weld therein, end members welded to opposite ends of said main body portion, one of said end members being formed of relatively hard material of substantially uniform hardness therethrough, the other of said end members and said main body portion having a greater carbon content in the exposed surface areas thereof than in the remainder thereof, said carbon content extending into said longitudinal weld, those portions only of said other end member and said main body portion including said greater carbon content being hardened.

5. A barrel type valve tappet comprising a hollow cylindrical body of substantially uniform diameter and uniform wall thickness throughout its length and the interior of which is hermetically sealed, one end of said body having a shouldered member of substantially the same external diameter as the cylindrical body adjacent the portion where it is welded thereto, the outer and inner axial portions of said member being of substantially reduced diameter, the outer of said axial portions having a relatively hard peripheral surface and a relatively soft interior, said interior of said outer axial portion being provided with a threaded blind opening therein, an adjusting screw received in said opening, and a member of harder characteristics than said body and the first mentioned member closing the opposite end of said body.

6. A barrel type valve tappet comprising a hollow cylindrical imperforate body portion of substantially uniform diameter and uniform wall thickness throughout its length, imperforate end walls of substantially the same external diameter as the body portion, welded in sealed relation to opposite ends of said body portion, one of said end walls having a blind threaded opening there-

in surrounded by internal surfaces of relatively soft character and exposed surfaces of relatively hard character.

- 5 7. A barrel type valve tappet comprising a hollow cylindrical body of substantially uniform diameter and wall thickness throughout its length, an annular shouldered end member having an annular wedge-shaped groove in one face thereof cooperatively received on one end of said body portion and welded thereto, and a second disc-like end member having an annular wedge-

shaped groove in one face thereof received by the opposite end of said body portion and welded thereto, said disc-like end member being of relatively hard character and of uniform hardness therethrough, the outer surface areas of said body portion and said shouldered end member being of relatively hard character and said body portion and said shouldered end member being of relatively soft character except for said surfaces.

5

10

JOSEPH H. HOERN.